

# UNITED STATES PATENT OFFICE.

ROBERT SWAIN PERRY, OF CAVE SPRING, GEORGIA.

## MANUFACTURE OF PAINTS.

938,505.

No Drawing.

Specification of Letters Patent.

Patented Nov. 2, 1909.

Application filed May 27, 1908. Serial No. 435,266.

To all whom it may concern:

Be it known that I, ROBERT SWAIN PERRY, of Cave Spring, in the county of Floyd and State of Georgia, (whose present post-office address is Queen and Stokely streets, Falls of Schuylkill, Philadelphia, in the county of Philadelphia and State of Pennsylvania,) have invented certain new and useful Improvements in the Manufacture of Paints, 10 whereof the following is a specification.

The object of my invention is to enable the production of paints, varnishes and stains, which shall have a positive power of retarding or inhibiting the rusting of steel and 15 iron surfaces upon which they may be applied.

In order to fully comprehend the scope and purpose of my invention, as thus indicated, it is necessary to briefly advert to certain characteristics of paints, as heretofore employed.

A paint, as known in the arts, is primarily an incorporation of a solid pigment, or pigments, in a more or less liquid vehicle, which 25 vehicle, after application upon a surface, will oxidize, dry, or otherwise harden so as to remain in intimate contact with the underlying surface, and to form a composite skin or protective coating therefor. Incidentally, 30 the paint, may of course, be required to have a decorative value, but, for the present purposes, this feature may be deemed negligible, since the protective feature, as such, is the subject for consideration. The protection 35 afforded to iron and steel by most paints is simply the indirect one of affording a covering, which tends to prevent the access of moisture and acids and other rust forming agencies; and in such aspect the desiderata 40 are that the vehicle and the solid ingredients carried thereby, shall be of such character as to prolong the physical integrity of the coating, and that they shall not either individually or as the result of combination, tend to 45 corrode the metallic surface to any substantial extent. Recently attempts have been made to employ pigments, or solid ingredients, in paints, which shall, in themselves, 50 tend to directly prevent or retard the corrosion of iron or steel, so as not merely to constitute a coating which tends to exclude moisture, but to counter-act to some extent the effect of such moisture as may actually penetrate to the iron or steel. As a convenient term, the expression "rust-inhibiting," 55 may be applied to such ingredients as pos-

sess the inherent quality of preventing or retarding the corrosion of iron or steel in the presence of moisture and moisture forming compounds.

The distinction between the vehicle and pigment is not only one recognized as fundamental in the paint making art, but, it is for the purpose now under consideration, of great practical importance, owing to the physical characteristics of the vehicle, which are liquid or semi-liquid, and those of the true pigmentary ingredients, which are of solid character, however fine may be the state of subdivision of their particles.

In order that I may clearly indicate my discovery and invention, it is necessary for me to classify the materials entering into paint, with regard to their solubility in water or in linseed oil, which, for practical purposes, may be considered as the typical substances important in this connection. For the purpose of such classification of pigmentary materials, it is proper to distinguish between insoluble materials (in either of the above mentioned liquids) slightly soluble materials, and freely soluble materials. An insoluble material would be one which would not to any appreciable extent be soluble in the liquids mentioned. The difference between slightly soluble materials and freely soluble materials may be defined as follows:—A pigmentary material, in which the particles have definite solid form, if treated by water or by linseed oil, in the proportion of these substances which would obtain in the use thereof in actual practice of the paint industry, would not, in the case of a slightly soluble material, substantially lose the form of its particles, as a whole, whereas, a freely soluble material would completely dissolve and wholly lose the solid form of its particles. Therefore, in the case of a slightly soluble material, in the above aspect, it may be said that although there might be a small percentage of the solid material taken up by the liquid, yet the portion actually dissolved would not be considered by a paint maker, as substantially modifying the formula of the resultant product.

Returning now to the use of rust inhibiting ingredients, so far as I am aware, they have usually been essentially a part of the pigment, or solid component carried by the vehicle, and have been either linseed oil insoluble, or linseed oil slightly-soluble, and at the same time either water slightly-solu-

ble or water freely-soluble, and the positive protection thus afforded, has limitations which it is the object of my invention to avoid.

5 I have found that the vehicle itself may be so constituted as to have a positive rust inhibiting tendency, irrespective of the character of the pigment or pigments carried thereby, and that by reason of this fact a 10 highly advantageous distribution and application of the desired properties can be obtained.

I have discovered that there is a class of positive rust inhibiting ingredients which 15 are freely linseed-oil soluble, and which may therefore be directly combined with the ordinary vehicles employed for paint in such a manner as not to substantially modify the essential character thereof. I believe this 20 rust-inhibiting action to be due to the fact that said ingredients have the property of decreasing the concentration of the hydrogen ions at the point of contact of moisture with the iron or steel surface, or that they 25 in some manner prevent the interchange of the electrostatic charge between said metal and the hydrogen ions; but, whether this theory be correct or not, the fact is that they do positively inhibit corrosion by preventing 30 or retarding the attack upon the iron or steel which results in rusting. Substances thus adapted for direct combination with the vehicle, should preferably have the following qualities:—They should not substantially 35 detract from the attributes of the vehicle in respect to its capacity for mechanically carrying the solid pigmentary ingredients; they should exhibit only a moderate tendency toward chemical reaction with the staple com- 40 mercial pigments, either in the direction of injuriously modifying said pigments, or of being themselves injuriously modified by the latter; and they should be such as not to substantially impair the color effect or homogeneuous appearance of the finished paint 45 coating.

The class of materials which I wish to include in this patent and to which I restrict my claims, are those combinations of an organic acid radical with an inorganic base (such as linoleate of chromium and resinate of chromium) which are rust inhibitors, and 50 which have the following characteristics; viz: that they are freely linseed-oil soluble, but not freely water soluble, as those terms are above explained, although they may be slightly water soluble as that term is above explained; further, that the metal of the base, in each case, is precipitable in ammoniacal solution, as a sulfid or hydrate, by means of hydrogen sulfid; further, that the metal of the base is electronegative to iron when placed in contact with iron and embedded in ferroxyl indicator; further, that 55 in the presence of distilled water they do

not electrically excite iron to any substantially greater extent than do similar compounds of chromium; finally, that these materials are compounds which, in the presence of distilled water and iron, have a tendency to disassociation substantially as low as that which is evident in the case of similar compounds of chromium. It will of course, be understood that a plurality of such ingredients may be employed together, 75 provided that each possesses the essential characteristics above set forth.

As a typical example of a process for preparing a rust-inhibiting ingredient and combining it with linseed oil I give the following:—One hundred pounds of linseed oil are saponified with nineteen pounds of caustic soda and the resultant product is treated with seventy-eight pounds of chrome alum, to precipitate about one hundred pounds of 80 chromium linoleate soap. As a typical process with a resin, one hundred pounds of rosin are saponified by the addition of twelve pounds of soda ash, and fifty pounds of chrome alum are added, to precipitate 85 about one hundred pounds of chromium resinate soap. The resultant product thus obtained may conveniently be employed to form an initial solution in linseed oil and such initial solution, with or without the 90 ordinary so-called thinners, may be combined with the vehicle, preferably in such quantity that the rust inhibiting product above described may constitute about five per cent. of the total material of the ultimate paint. This paint of course may be thinned down to the proper consistency in the usual manner with oil or with varnish, turpentine, or other thinners. The percentage of rust-inhibiting ingredient however, may be varied, depending upon the 95 following condition.

It is known that pigments have in some instances a tendency to produce rust, in other instances they are practically inert in that 100 respect, and in other instances they have positive rust inhibiting tendencies. According therefore to the inherent character of the pigmentary material in this respect, a greater amount than that before stated may 105 be employed where the pigment itself is a rust producer, or a less amount may be used where the pigment is a rust-inhibitor, the percentage named being a convenient one for use in connection with a practically inert 110 pigment.

I am aware that it has heretofore been suggested to employ rust-inhibiting ingredients as a part of a liquid or semi-liquid vehicle, but in such instances, they have consisted entirely of inorganic compounds, such as potassium bichromate and chromate of zinc, or of compounds in which the acid radical is inorganic, and in these cases the positive protection afforded by their use has 115 120 125 130

limitations which it is the object of my invention to avoid.

In the above description I have referred to paints as the most prominent and important products to which my invention is adapted, but it will be understood that the rust inhibiting ingredients of the class comprehended may be employed in connection with varnishes or stains, in which solid pigmentary ingredients are not essential, hence I class these products as of like character with the paints for the purposes and scope of my invention. Furthermore, it will be understood that my invention does not exclude the use of rust-inhibiting pigmentary material, and that hence in stating that the rust-inhibiting qualities of paints, or the like, in which my invention is employed, are owing to the presence of the described ingredients, I mean that such qualities may be due either wholly or in part to the presence thereof.

Having thus described my invention, I claim:

1. A rust-inhibiting paint or the like, owing its rust-inhibiting qualities to an organic acid radical combined with an inorganic base, such compound being freely lin-

seed-oil-soluble, but not freely water-soluble, and having the characteristics that the metal of its base is precipitable in ammoniacal solution, as a sulfid or hydrate, by means of hydrogen sulfid; further, that the metal of its base is electronegative to iron, when placed in contact with iron and embedded in ferroxyl indicator; further, that in the presence of distilled water it does not electrically excite iron to any substantially greater extent than do similar compounds of chromium; finally, that in the presence of distilled water and iron it has a tendency to disassociation substantially as low as that which is characteristic of chromium resinate.

2. A rust-inhibiting vehicle for paint or the like, consisting of a chromium base combined with an organic acid radical, such compound being freely linseed-oil-soluble, but not freely water-soluble, substantially as set forth.

In testimony whereof, I have hereunto signed my name, at Philadelphia Pennsylvania this twenty-sixth day of May 1908.

ROBERT SWAIN PERRY.

Witnesses:

F. ASHWORTH,  
P. H. BUTLER.

Correction in Letters Patent No. 938,505.

It is hereby certified that in Letters Patent No. 938,505, granted November 2, 1909, upon the application of Robert Swain Perry, of Cave Spring, Georgia, for an improvement in the "Manufacture of Paints," an error appears in the printed specification requiring correction, as follows: Page 2, line 30, the word "ion" should read "iron"; and that the said Letters Patent should be read with this correction therein that the same may conform to the record of the case in the Patent Office.

Signed and sealed this 30th day of November, A. D., 1909.

[SEAL.]

E. B. MOORE,  
*Commissioner of Patents.*

limitations which it is the object of my invention to avoid.

In the above description I have referred to paints as the most prominent and important products to which my invention is adapted, but it will be understood that the rust inhibiting ingredients of the class comprehended may be employed in connection with varnishes or stains, in which solid pigmentary ingredients are not essential, hence I class these products as of like character with the paints for the purposes and scope of my invention. Furthermore, it will be understood that my invention does not exclude the use of rust-inhibiting pigmentary material, and that hence in stating that the rust-inhibiting qualities of paints, or the like, in which my invention is employed, are owing to the presence of the described ingredients, I mean that such qualities may be due either wholly or in part to the presence thereof.

Having thus described my invention, I claim:

1. A rust-inhibiting paint or the like, owing its rust-inhibiting qualities to an organic acid radical combined with an inorganic base, such compound being freely lin-

seed-oil-soluble, but not freely water-soluble, and having the characteristics that the metal of its base is precipitable in ammoniacal solution, as a sulfid or hydrate, by means of hydrogen sulfid; further, that the metal of its base is electronegative to iron, when placed in contact with iron and embedded in ferroxyl indicator; further, that in the presence of distilled water it does not electrically excite iron to any substantially greater extent than do similar compounds of chromium; finally, that in the presence of distilled water and iron it has a tendency to disassociation substantially as low as that which is characteristic of chromium resinate.

2. A rust-inhibiting vehicle for paint or the like, consisting of a chromium base combined with an organic acid radical, such compound being freely linseed-oil-soluble, but not freely water-soluble, substantially as set forth.

In testimony whereof, I have hereunto signed my name, at Philadelphia Pennsylvania this twenty-sixth day of May 1908.

ROBERT SWAIN PERRY.

Witnesses:

F. ASHWORTH,  
P. H. BUTLER.

Correction in Letters Patent No. 938,505.

It is hereby certified that in Letters Patent No. 938,505, granted November 2, 1909, upon the application of Robert Swain Perry, of Cave Spring, Georgia, for an improvement in the "Manufacture of Paints," an error appears in the printed specification requiring correction, as follows: Page 2, line 30, the word "ion" should read "iron"; and that the said Letters Patent should be read with this correction therein that the same may conform to the record of the case in the Patent Office.

Signed and sealed this 30th day of November, A. D., 1909.

[SEAL.]

E. B. MOORE,  
*Commissioner of Patents.*

It is hereby certified that in Letters Patent No. 938,505, granted November 2, 1909, upon the application of Robert Swain Perry, of Cave Spring, Georgia, for an improvement in the "Manufacture of Paints," an error appears in the printed specification requiring correction, as follows: Page 2, line 30, the word "ion" should read *iron*; and that the said Letters Patent should be read with this correction therein that the same may conform to the record of the case in the Patent Office.

Signed and sealed this 30th day of November, A. D., 1909.

[SEAL.]

E. B. MOORE,  
*Commissioner of Patents.*